# EUROPEAN PATENT APPLICATION

(11) **EP 0 444 642 A1**
(43) Date of publication of application: **04.09.1991**
(21) Application number: 91102940.3
(22) Date of filing: 27.02.1991
(51) Int. Cl.: C23C 12/02

(54) **A method of obtaining a diffusion protective coating on ferrous alloys**

(30) Priority: 28.02.1990 PL 284129
(71) Applicant: INSTYTUT CHEMII NIEORGANICZNEJ, PL-44-101 Gliwice (PL)
(72) Inventor: Generalczyk, Krzysztof, Poznán (PL); Jakubowski, Jan, Poznán (PL); Mlynarczak, Andrzej, Poznán (PL)
(74) Representative: von Füner, Alexander, Dr.

(57) **Abstract**

This invention is related to a method of obtaining an anti-corrosive acid-resisting protection on ferrous alloys, particularly against the effect of sulfuric acid, in heat treatment processes by way of subjecting them to the diffusive effect of the silicon and boron compositions, which is characterized by the fact that ferrous alloys of the carbon content being not lower than 0.12% are placed into a mixture in which the weight ratio of the active silicon compounds to the active boron compounds is at least equal to zero, and so selected that the protective coating would contain the Fe_{α}/Si solution and intermetallic stages of the minimum participation of boron.

## Description

The subject of the present invention is a method of obtaining an anti-corrosive protective coating on ferrous alloys, being simultaneously acid- and heat-resisting protection, whereas the acid-resisting protection, particularly against the effect of sulfuric acid at high temperatures, is obtained when ferrous alloys are subjected to the diffusive action of the silicon- and boron-containing mixture.

There is known a method of protecting the steel against the corrosive effect of sulfuric acid by applying an anodic coating. The said method, being quite complicated as far as the equipment is concerned, at the temperature of above 100°C provides an effective protection only for the high-alloy steel.

There are also known the methods of obtaining the acid-resisting protection of steel by applying thereupon the sprayed coatings of plastics or of a metallic layer of zirconium, tantalum or chromium. The plastics coatings effectively protect the steel against sulfuric acid at low temperatures, below 80°C. The zirconium coatings protect the steel only against the effect of sulfuric acid of the concentrations below 70% by weight. It is very expensive to obtain protection with the aid of tantalum, whereas in order to obtain the protection of steel as per the Polish patent specification No. 146144, by applying the sprayed protective coating, there is required a troublesome pre-treatment, and it only provides the effective protection against the acid of the high concentration ranging above 98.3% by weight.

From the publication N. Gorbunow "Diffuzionnyje pokrytija na zelezie i stali", Izd. AN SSSR, Moscow, 1958, there are known acid- and heat-resisting protective coatings as obtained by diffusively enriching the surface layer of steel with silicon. They are advatageous because of their increased resistance against the corrosion effected by various acids and because of their heat-resistance up to 800°C.

There is known a method to obtain the anti-corrosive protection of metals by way of diffusively applying the protective coatings in the heat-treatment process by placing a worked piece into appropriate mixtures of powders which, inter alia, contain chromium, aluminum, silicon or boron, being applicable for obtaining single or double-layer coatings, whereas the latter are obtained by additionally applying, for instance, boron upon the particular Al, Si or Cr coatings.

Besides the application of one-constituent layers of coatings there are also known the coatings being obtained by the simultaneous application of two constituents.

Into the sets of mixtures which according to the USSR patents No. 718496 and No. 819216 are suited for the application of coatings by way of the simultaneous diffusive boron-silicvon impregnation of ferrous alloys, the active boron compounds are in excess as compared to silicon compounds because the silicon being added particularly in the form of the non-active SiO₂ serves only as a modifier accelerating the diffusion processes. The said mixtures also contain other activators and fillers. The aim of producing the coatings being obtained in the course of the boron-silicon impregnation into the mixtures with the excess of boron compounds, said coatings mainly containing FeB and Fe₂B stages, is their hardness and abrasion resistance, because the too high content of silicon compounds into the mixture causes the thickness of the layer of borides get decreased and their abrasion resistance be diminished.

In the course of the testings as carried out over the protective coatings being obtained on ferrous alloys before the corrosive effect of the oxidizing medium, acids inclusively, it appeared that the acid resistance of the Si-B coatings being obtained according to the method as per the present invention is many times higher than the acid resistance of the B, Si, Cr, Cr-Si, Ni-Cr and Ni-B coatings being tested parallelly.

The essence of the solution as per the present invention is a method of obtaining an anti-corrosive, protective coating, particularly an acid-resisting and simultaneously heat-resisting one, upon ferrous alloys by way of diffusively applying the said coating in the course of the heat treatment process by placing the worked piece into a powdered mixture containing the silicon- and boron-bearing compounds together with an activator and a filler. The said process is characterized by the fact that the ferrous alloys of the carbon content into the steel being not lower than 0.12% are placed into the mixture in which the ratio of active silicon compounds to active boron compounds, being by weight at least equal to one, is so selected that the underlayers of the coating, containing the intermetallic stages of Fe and silicon, be only modified with boron. The coating which is built up of the underlayers of varied morphology contains the Fe_{α}/Si and intermetallic stages of the Fe-Si system with the minimum participation of boron.

### EXAMPLE:

Kaolin which was, in order to get dehydrated, in the course of 2 hourse subjected to roasting at a temperature of 200°C, was mixed into a drum mixer with ferrosilicon, being the source of the highly active silicon, and beforehand screened through a 0.075 mm mesh sieve, and mixed with boron carbide being the source of active boron in the wieght ratio of 40:30:30. Furthermore, into the said mixture aluminium fluoride in the amount of 0.5% by weight of the mixture was added as an activator. Samples of steel 20 together with the formerly prepared powdered mixture were placed into an air-tight retort being constructed so that the samples of steel as placed therein did not contact each other and were not in contact with the walls of the retort. The said retort was heated up into a silite furnace at a temperature of 950°C in the course of 5 hours. After the retort was cooled and discharged, the samples were cleaned from powder residues.

In other variants of this example of embodiment, instead of kaolin, being the source of the non-active silicon, quartz was applied as a filler, whereas as an activator there were variously used aluminium, ammonium or potassium fluorides or chlorides. Moreover, the steels of the carbon content being lower than 0.12% were subjected to carbonization before being boron-silicon impregnated. The powdered mixture containing the varied active compounds of silicon and boron, being applied into the method as per the present invention, may be many times utilized in subsequent processes of the boron-silicon impregnation and only the periodical making up of the activator is required, in the amount as usually added to the fresh powder. The thus obtained thickness of the coating was 0.4 mm. The said coating, under the post-structure surface layer of 300 µm, comprises the two relatively compact layers, the external one being 200 µm thick and the internal one being 100 µm thick, and further on the porous internediate layers. In the quantitaive analysis it has been shown that the worked layers are significantly enriched with Si, that the intermetallic layer being obtained accordingly to the method as described in this example is in the form of Fe₃Si, and furthermore, that the Fe_{α}/Si solution occurs therein.

After this test controlling the acid resistance of the coating obtained was carried out, when the samples were subjected to the effect of the hot sulfuric acid within the temperature range of 150 to 285°C in the course of 2000 hours, there were not stated any changes into the surface of the samples.

The scale as obtained upon the sample being subjected to the heat resistance test at the temperature of 800°C in the course of 120 hours is characterized by the compactness and high adhesion.

## Claims

1. A method of obtaining a diffusion anti-corrosive protective coating on ferrous alloys, particularly acid-resisting and simultaneously heat-resisting one, by the application of a coating in the process of heat treatment by way of placing the worked piece into a powdered mixture which contained compounds being the source of boron and silicon, and an activator and a filler, characterized in that the ferrous alloys of the carbon content in the steel being not lower than 0.12 % are placed into the mixture in which the ratio of the active silicon compounds to the active boron compounds, being by weight at least equal to one, is so selected that the coating which is built up of the underlayers of varied morphology contained Fe_{α}/Si solution and intermediate stages of the Fe-Si system with the minimum participation of boron.
